

## MIXED METAL COMPLEX SALTS OF PHOSPHORIC ACID ESTERS AND MINERAL OIL COMPOSITIONS CONTAINING THE SAME

Ferdinand P. Otto, Woodbury, N. J., and Edmund W. Flynn, Urbana, Ill., assignors to Socony Mobil Oil Company, Inc., a corporation of New York

No Drawing. Application October 20, 1955,  
Serial No. 541,848

20 Claims. (Cl. 252—32.5)

This application is a continuation-in-part of copending application Serial No. 246,502, filed September 13, 1951, now abandoned.

This invention relates to improved lubricating oil compositions, particularly mineral lubricating oils for use in internal combustion engines.

As is well known, mineral lubricating oils refined for use as lubricants have a tendency to oxidize in use in an engine with attendant formation of oxidized products which are acidic in character and which exert a strong corrosive action on the engine parts, such as the hard metal alloy bearings. The oxidation of the oil also produces carbonaceous sludge deposits in the engine, particularly around the pistons and oil rings causing them to stick, thus materially lowering the efficiency of the engine.

To counteract these conditions, there have been developed in the art chemical agents which when added to a mineral lubricating oil designed for use in internal combustion engines, have the ability to inhibit or retard oxidation of the oil. These agents are designated as antioxidants. Other agents have been developed which have the ability to suspend the carbonaceous oxidation products formed in the oil, thereby keeping the engine parts clean and free from clogging and sticking effects normally encountered. These materials are known as detergents. The present invention is concerned with chemical additives which exhibit a two-fold ability, viz., (1) the ability to inhibit the formation of acidic, corrosive oxidation products in the oil during use in an engine and (2) the ability to keep the engine parts clean and free from sticking. These additives are, therefore, antioxidants as well as detergents. This two-fold action of these materials is, of course, of great advantage from an economic standpoint since ordinarily separate additives are employed to impart each of these characteristics to an oil.

It is, therefore, the object of this invention to provide a mineral lubricating oil composition which is stabilized against the formation of corrosive bodies therein during use and which is also fortified as to its detergent ability. Other and further objects will appear from the following detailed description of the invention.

The additives contemplated herein may be designated, broadly, as "mixed-metal," zinc-containing, complex salts of partial esters of phosphoric acid. Due to the complex nature of these compounds, their exact chemical structures are not presently known.

Broadly, the complex salts of the invention are prepared by the method which comprises the steps of (1) reacting one mol of phosphorus pentoxide with from about one to about three mols of an organic hydroxy compound selected from the group consisting of a hydroxyaromatic compound that has an alkyl substituent having at least 8 carbon atoms in place of a nuclear hydrogen atom thereof and a primary, aliphatic alcohol having at least 8 carbon atoms per molecule, to form an acidic, partial ester of phosphoric acid, (2) reacting said acidic partial

ester of phosphoric acid with a zinc salt reagent in an amount sufficient to furnish at least one equivalent of zinc per equivalent of acid-hydrogen content in said acidic, partial ester of phosphoric acid, and (3) reacting the product obtained in step 2 with a metal hydroxide selected from the group consisting of calcium hydroxide, barium hydroxide, strontium hydroxide, cadmium hydroxide, magnesium hydroxide and cobalt hydroxide, in an amount sufficient to furnish at least one equivalent of metal per equivalent of acid-hydrogen content in said acidic, partial ester of phosphoric acid.

In the practice of the invention, the reaction of the partial ester with the metal salt reagent can be accomplished by first reacting about one equivalent of a zinc salt, such as zinc hydroxide, zinc carbonate, zinc alcololate or a zinc carboxylate, followed by reaction with at least one equivalent of a metal hydroxide of a metal selected from calcium, barium, strontium, cadmium, magnesium and cobalt. However, more than one equivalent 15 of the zinc salt reagent, other than zinc hydroxide, can be used in the first reaction, say, up to and including two equivalents, or more, followed by reaction with at least an additional equivalent amount of the metal hydroxide other than zinc. It will be understood, therefore, that 20 the one equivalent of each of the two different metal salts actually represents the minimum amounts of these reagents which can be employed. Alternatively, the reaction of the partial ester with the metal salt reagent can be conducted by utilizing at least about two equivalents of a zinc carboxylate reagent in the first reaction followed by reaction with at least an additional equivalent of a metal hydroxide reagent selected from the metal hydroxide of calcium, barium, strontium, cadmium, magnesium and cobalt. Here again, these amounts represent 25 the minimum amounts of these reagents which can be used. Thus, although higher amounts than those stipulated for the various reagents can be used, such amounts will provide no particular advantage. It can be said then that the upper limit with respect to the amounts of 30 the several metal reagents is not a critical factor but is governed largely by practical considerations. Thus, for example, the use of large excess amounts of the metal reagents tends to reduce the fluidity of the reaction mass, thereby creating handling and filtration difficulties.

40 The total amount of metal which is incorporated into the complex salts of the invention is usually from two to three times, or more, greater than that which would be contained in the normal salts of the partial esters. Due to their high metal contents, these "mixed-metal" complex 45 salts possess superior properties as oil detergents over the normal salts. It will be appreciated that the complex salts prepared by the use of two equivalents, or more, of a zinc carboxylate followed by reaction with an additional equivalent of metal hydroxide are actually 50 complexes of complex zinc salts having an added metal content of a different metal. The complex zinc salts are disclosed and claimed as mineral oil additives and as new 55 compositions of matter in a copending application, Serial No. 541,849, filed October 20, 1955, in the name of 60 Ferdinand P. Otto, one of the applicants herein.

It is recognized that normal salts of phosphoric acid esters have been disclosed heretofore as oil additives, e. g., they are shown in U. S. Patents Nos. 2,228,658 and 2,228,659 to B. B. Farrington and No. 2,228,271 to 65 George L. Neeley. However, as far as is known, there has been no disclosure in the art of mixed-metal complex salts of the character herein contemplated. Since these salts per se have not been known heretofore, they are claimed herein as new compositions of matter.

70 As previously stated, the reactions involved in the formation of the mixed-metal salts of the invention are complicated and the exact structure of these compounds have

not been determined. Theoretically, however, it is known, with respect to the phosphoric acid esters, that when an alkylated hydroxyaromatic compound, such as an alkylphenol (or a primary, aliphatic alcohol), reacts with phosphorus pentoxide in a mol ratio of 3:1, for example, the product consists essentially of a mixture of (1) monoalkaryl (or -alkyl) phosphoric acids, (2) di-alkaryl (or-alkyl) phosphoric acids and (3) pyrophosphoric acids. These compounds are represented by the following formulae in which R represents the organic substituent.

(1)



(2)



(3)



The mol ratio of the hydroxy reactant to phosphorus pentoxide would, of course, be expected to affect the relative proportions of these compounds present in the product mixture. When, for example, this mol ratio is 3:1, the major components of the product are believed to be the mono- and di-esters of phosphoric acid with minor amounts of pyrophosphoric acid.

It has been found that when a normal zinc salt of, for example, the octylphenol-phosphorus pentoxide (3:1) product is further reacted with a hydroxide of a metal such as calcium, barium, strontium, cadmium, cobalt or magnesium, a product salt is formed, which contains up to as many as three equivalents of total metal, including zinc, per equivalent of acidity in the octylphenol-phosphorus pentoxide product. As aforesated, the exact structure of such complex salt products is not known. However, it is believed that the extra equivalents of metal are incorporated into the molecule through a coordination or complexing of the metal hydroxide with the normal zinc salt of the phosphoric acid ester. Thus, the reaction of magnesium hydroxide with the normal zinc salt of the octylphenol-phosphorus pentoxide product might, for example, occurs as follows:



#### ALKYL HYDROXYAROMATIC COMPOUND

The preparation of the compounds of the invention involves, first, the alkylation of a hydroxyaromatic compound, such as phenol, i. e., where an alkaryl phosphoric acid ester is desired. This may be accomplished by methods known to the art, such as by a Friedel-Crafts synthesis using a halogenated hydrocarbon. The alkylation may also be effected by reaction of the aryl hydroxide with unsaturated hydrocarbons, or alcohols, in the presence of sulfuric acid as a catalyst.

Typical aryl hydroxides which may be used as the starting material for the alkylation reaction are: phenol, resorcinol, hydroquinone, catechol, cresol, xylenol, hydroxydiphenyl, benzyl-phenol, phenyl-ethyl-phenol, phenol resins, methyl-hydroxydiphenyl, guaiacol, alpha and beta naphthol, alpha and beta methyl naphthol, tolyl naphthol, xylyl naphthol, benzyl naphthol, anthranol, phenyl methyl naphthol, phenanthrol, chlorophenol and the

like. Preference in general is to the monohydroxy phenols otherwise unsubstituted, particular preference being given to phenol and alpha and beta naphthol.

The hydroxyaromatic compound may have one or several alkyl groups attached to the nucleus thereof. In any case, the alkyl portion of this compound should contain a total of at least 8 carbon atoms. Thus, if the alkyl substituent contains less than 8 carbon atoms, the aromatic nucleus should contain more than one such substituent to bring the carbon atom content of the side chains so attached to about 8 in order to provide ultimate complex salts which are completely oil-soluble. On the other hand, the hydrocarbon from which the alkyl group is derived may suitably contain up to 30 or even 40 carbon atoms.

In fact, a highly suitable source of the alkyl substituent is petroleum wax which contains hydrocarbon molecules having from about 20 to about 30 carbon atoms and an average of about 24 carbon atoms per molecule. Other suitable alkyl hydroxyaromatic compounds are, for example, octylphenol, diethylphenol, decylphenol, laurylphenol, tetradecylphenol, hexadecylphenol and octadecylphenol, octylphenol being particularly preferred.

Where an aliphatic alcohol is used for reaction with the phosphorus pentoxide, rather than an alkaryl hydroxy compound, it should likewise contain at least about 8 carbon atoms and suitably as high as 20 or 30 carbon atoms. Of the alcohols suitable for use in the invention, there may be mentioned as non-limiting examples the following: octyl alcohol, nonyl, decyl, undecyl, dodecyl, tetradecyl, hexadecyl, octadecyl, carnaubyl, cetyl and melissyl alcohols. Unsaturated alcohols, such as oleyl alcohol, may also be used.

The various alkylphenols and aliphatic alcohols utilized in the invention, with the exception of the wax-alkylated phenols, are either available commercially or the methods for their preparation are within the skill of those versed in the art. The preparation of a wax-alkylated type of product, however, is illustrated by the following procedure.

#### WAX-PHENOL

A paraffin wax melting at approximately 120° F. and



predominantly comprised of hydrocarbons, having at least 20 and an average of about 24 carbon atoms in their molecules, is melted and heated to about 200° F., after which chlorine is bubbled therethrough until the wax has absorbed about 14%, by weight, of chlorine. A sufficient quantity of this chlorinated wax to provide three atomic proportions of chlorine is then heated to a temperature varying from just about its melting point to not over 150° F. One mol of phenol ( $\text{C}_6\text{H}_5\text{OH}$ ) is then mixed with the chlorowax. The mixture is then heated to about 150° F. and a quantity of anhydrous aluminum chloride, corresponding to about 3% of the weight of the chlorowax in the mixture, is slowly added with active stirring. The rate of addition of the aluminum chloride should be sufficiently slow to avoid violent foaming and during the addition the temperature should be held at about 150° F. After the aluminum chloride has been added, the temperature of the mixture may be increased slowly over a

period of 15 to 25 minutes to a temperature of about 250° F. and then should be more slowly increased to about 350° F. To control the evolution of HCl gas, the temperature of the mixture is preferably raised from 250° F. to 350° F. at a rate of approximately one degree per minute, the whole heating operation occupying approximately two hours from the time of adding the aluminum chloride. If the emission of HCl gas has not ceased when the final temperature is reached, the mixture may be held at 350° F. for a short time to allow completion of the reaction. However, to avoid possible cracking of the wax, the mixture should not be heated appreciably above 350° F., nor should it be held at that temperature for any extended length of time.

It is important that all unreacted, or non-alkylated, phenol remaining in the reaction mixture, as well as aluminum chloride, be removed. This can be conveniently effected by washing the product several times with a mixture of water and an alcohol, such as butanol, preferably at elevated temperature, say 175° F. The product may then be treated with steam. This latter step will insure complete removal of the unreacted material and also dry the product.

It will be understood that a wax-substituted phenol prepared according to the above procedure, in which a quantity of chlorowax containing three atomic proportions of chlorine and having a chlorine content of 14% is reacted with one mol of phenol, is designated as "wax-phenol (3-14)." Similarly, "wax-phenol (3-10)" and "wax-phenol (1-10)" may also be prepared by the reaction of sufficient amounts of chlorinated wax, containing 10% by weight of chlorine, to provide three atomic proportions and one atomic proportion of chlorine per mol of phenol, respectively, in the reaction and are useful in the invention. In general, the amount of chlorowax, containing from about 10% to 18% by weight of chlorine, used in the reaction is sufficient to supply between one and four atomic proportions of chlorine per mole of phenol used.

#### PARTIAL ESTER OF PHOSPHORIC ACID

In preparing the phosphoric acid ester, the phosphorus pentoxide and the alkyl hydroxyaromatic compound, or alcohol, are heated together at a temperature of from about 50° C. to about 150° C. for a period of time to insure substantially complete reaction, usually from about 5 to 15 hours. An inert solvent, such as toluene, xylene or the like, may be used to facilitate the reaction. A mineral oil may also be conveniently used as the solvent, in which case the product is an oil concentrate which may be used directly in the preparation of the ultimate complex mixed-metal salt. In this way, the complex salt product is obtained in the form of an oil concentrate and may be utilized as such for addition to mineral lubricating oils. Where a solvent other than mineral oil is used, the reaction mixture is filtered and topped at elevated temperature and reduced pressure to remove the solvent.

The proportion of alkyl hydroxyaromatic compound, or alcohol, and phosphorus pentoxide used in the reaction can be varied between from about one to about three mols of the alkyl hydroxyaromatic compound, or alcohol, to one mol of phosphorus pentoxide, although our preferred products are obtained by the use of about three mols of the alkyl hydroxyaromatic compound (or alcohol) per mol of phosphorus pentoxide.

#### MIXED-METAL COMPLEX SALT

As indicated previously, the mixed-metal complex salts can be prepared from the normal zinc salts of the partial esters of phosphoric acid by reaction with a metal hydroxide of the metals calcium, barium, strontium, cadmium, magnesium and cobalt. Mixed-metal complex salts can also be made, however, without first forming a

normal salt, by first forming the complex zinc salt and then further complexing the complex zinc salt by reaction with one of the said metal hydroxides.

The reaction between the phosphoric acid ester and zinc salt reagent to form the normal zinc salt or the complex zinc salt and the reaction between either of these and the metal hydroxide to form the mixed-metal complex salt are accomplished at temperatures from about 50° C. to about 200° C. and are completed in a relatively short time, generally from about one-half hour to two hours. They may be carried out in a suitable solvent medium, such as benzene, toluene, xylene and the like, or a mineral oil may be used as the solvent.

As indicated previously, the amount of metal supplied to the reaction by the metal hydroxide when reacting it with either the normal zinc salt or the complex zinc salt should be sufficient to supply at least one additional equivalent of metal to the reaction based on the acid-hydrogen content of the partial ester used to make the normal salt. The amount of zinc acetate used to form the complex zinc salt, on the other hand, should be such as to supply at least two equivalents of zinc on the basis of the acid-hydrogen content of the partial ester used.

We have found that the formation of the mixed-metal complex salts is greatly enhanced by the presence in the reaction of a small amount of water in the reaction mixture. We have also found that in forming the complex zinc acetate salt, it is convenient and economical to supply the zinc acetate to the reaction as zinc oxide and acetic acid.

A full understanding of the nature and manner of preparation of the mixed-metal complex salts of the invention and their utility as oil additives may be had from the following illustrative examples and test results.

35

#### Example 1

##### OCTYLPHENOL-P<sub>2</sub>O<sub>5</sub> (3:1) PRODUCT

| 40 | Reaction mixture:             | Grams |
|----|-------------------------------|-------|
|    | Octylphenol                   | 800   |
|    | P <sub>2</sub> O <sub>5</sub> | 180   |

*Procedure.*—The octylphenol was placed in a 2 liter, 4-necked, round-bottom flask equipped with a reflux condenser, thermometer and mechanically driven stirrer and was heated to 100° C. with agitation. The temperature was maintained at 100° C. ±5° C. during portionwise addition of phosphorus pentoxide over a two-hour period and during the reaction period proper of eight hours duration. The clear light amber reaction product was filtered through filtering clay contained on a heated Buchner funnel. The product had an N. N. (neutralization number) of 210 and contained 7.99% phosphorus.

55

#### Example 2

##### NORMAL ZINC SALT OF OCTYLPHENOL-P<sub>2</sub>O<sub>5</sub> (3:1) PRODUCT

| 60 | Reaction mixture:                                                         | Grams |
|----|---------------------------------------------------------------------------|-------|
|    | Otetylphenol-P <sub>2</sub> O <sub>5</sub> (3:1) (Ex. 1)                  | 400   |
|    | Mineral oil (S. U. V. of 100 sec. at 100° F., acid-refined Mid-Continent) | 800   |
| 65 | ZnCO <sub>3</sub>                                                         | 94    |

*Procedure.*—The octylphenol-phosphorus pentoxide (3:1) product and the mineral oil were placed in a 3-liter, 4-necked, round-bottom flask equipped with a reflux condenser, thermometer and mechanically driven stirrer. The zinc carbonate was added gradually over a 15-minute period and the mixture heated to and maintained at 100° C. for two hours. The reaction product was filtered through filtering clay contained on a heated Buchner funnel giving a product containing 3.90% zinc.

## Example 3

COMPLEX CALCIUM-ZINC SALT OF OCTYLPHENOL-P<sub>2</sub>O<sub>5</sub> (3:1) PRODUCT

## Reaction mixture:

|                                                                                                                                                                                           |             |     |
|-------------------------------------------------------------------------------------------------------------------------------------------------------------------------------------------|-------------|-----|
| Normal zinc salt of octylphenol-P <sub>2</sub> O <sub>5</sub> (3:1) product (similar to Ex. 2) (containing 47% mineral oil [S. U. V. of 100 sec. at 100° F., acid-refined Mid-Continent]) | grams       | 400 |
| Ca(OH) <sub>2</sub>                                                                                                                                                                       | do          | 25  |
| H <sub>2</sub> O                                                                                                                                                                          | milliliters | 75  |

*Procedure.*—The zinc salt of octylphenol-phosphorus pentoxide (3:1) product was added to a 1-liter, 4-necked, round-bottom flask equipped with a condenser, thermometer and mechanically driven stirrer and heated at 65° C. The calcium hydroxide and water were added as a slurry to the reaction flask. The water was removed by distillation with the aid of a nitrogen flush by heating to a temperature of 150° C. which was attained in two hours. After cooling to 100° C., the filtering clay was added and the product filtered through filtering clay contained on a heated Buchner funnel. The filtrate, representing the finished product, contained 2.6% calcium and 4.26% zinc.

## Example 4

COMPLEX ZINC ACETATE SALT OF OCTYLPHENOL-P<sub>2</sub>O<sub>5</sub> (3:1) PRODUCT

## Reaction mixture:

|                                                                                   |             |      |
|-----------------------------------------------------------------------------------|-------------|------|
| Octylphenol-P <sub>2</sub> O <sub>5</sub> (3:1) product (Ex. 1)                   | grams       | 400  |
| Mineral oil (S. U. V. of 100 sec. at 100° F., acid-refined Mid-Continent)         | grams       | 800  |
| Zn(C <sub>2</sub> H <sub>3</sub> O <sub>2</sub> ) <sub>2</sub> .2H <sub>2</sub> O | do          | 329  |
| Ethyl alcohol, Formula 30 <sup>1</sup>                                            | milliliters | 1450 |

<sup>1</sup> A denatured alcohol containing 10 gallons of pure methanol per 100 gallons of 190° proof ethyl alcohol.

*Procedure.*—The octylphenol-phosphorus pentoxide (3:1) product and the mineral oil were placed in a 5-liter, 4-necked, round-bottom flask equipped with a reflux condenser, thermometer and mechanically driven stirrer and were heated with agitation to 70° C. The



was dissolved in the Formula 30 alcohol and the solution was added at 60° C. to the reaction flask. The mixture was then heated to 165° C. allowing alcohol and aqueous acetic acid to distill. After three hours at this temperature, the last two hours under diminished pressure, the reaction product was filtered through filtering clay contained on a heated Buchner funnel. The filtrate contained 8.35% zinc and 2.73% phosphorus.

## Example 5

COMPLEXED MAGNESIUM-ZINC ACETATE SALT OF OCTYLPHENOL-P<sub>2</sub>O<sub>5</sub> (3:1) PRODUCT

## Reaction mixture:

|                                                                                                                                                                                         |             |     |
|-----------------------------------------------------------------------------------------------------------------------------------------------------------------------------------------|-------------|-----|
| Complex zinc acetate salt of octylphenol-P <sub>2</sub> O <sub>5</sub> (3:1) product (Ex. 4) (containing 42% mineral oil [S. U. V. of 100 sec. at 100° F., acid-refined Mid-Continent]) | grams       | 600 |
| Mg(OH) <sub>2</sub>                                                                                                                                                                     | do          | 57  |
| H <sub>2</sub> O                                                                                                                                                                        | milliliters | 200 |

*Procedure.*—The zinc acetate salt of octylphenol-phosphorus pentoxide (3:1) product was added to a 2-liter, 4-necked, round-bottom flask equipped with a condenser, thermometer and mechanically driven stirrer and heated to 35° C. The magnesium hydroxide and water were added as a slurry to the reaction flask. The water was removed by distillation with the aid of a nitrogen flush by heating to a temperature of 165° C. The reaction mixture was then held at this temperature for one-half hour under diminished pressure. After cooling the product

75 N. N. of 158.

was filtered through filtering clay contained on a heated Buchner funnel. The filtrate, representing the finished product, contained 2.34% magnesium and 9.85% zinc.

## Example 6

DI-TERT-AMYLPHENOL-P<sub>2</sub>O<sub>5</sub> (3:1) PRODUCT

| Reaction mixture:             | Grams |
|-------------------------------|-------|
| Di-tert-amylphenol            | 2000  |
| P <sub>2</sub> O <sub>5</sub> | 405   |

*Procedure.*—The di-tert-amylphenol was placed in a 5-liter, 4-necked, round-bottom flask equipped with a reflux condenser, thermometer and mechanically driven stirrer. After heating to 100° C., phosphorus pentoxide was gradually added over a six-hour period. The reaction mixture was then held between 90° C. and 100° C. for eight hours to insure complete reaction. The reaction product was filtered through filtering clay contained on a heated Buchner funnel. The filtrate, representing the finished product, contained 7.40% phosphorus and had an N. N. of 183.

## Example 7

COMPLEX MAGNESIUM-ZINC ACETATE SALT OF DI-TERT-AMYLPHENOL-P<sub>2</sub>O<sub>5</sub> (3:1) PRODUCT

## Reaction mixture:

|                                                                                   |             |     |
|-----------------------------------------------------------------------------------|-------------|-----|
| Di-tert-amylphenol-P <sub>2</sub> O <sub>5</sub> (3:1) product (similar to Ex. 6) | grams       | 400 |
| Mineral oil (S. U. V. of 100 sec. at 100° F., acid-refined Mid-Continent)         | grams       | 564 |
| Zinc oxide                                                                        | do          | 107 |
| Acetic acid (glacial)                                                             | do          | 158 |
| Magnesium hydroxide                                                               | do          | 76  |
| H <sub>2</sub> O                                                                  | milliliters | 300 |

*Procedure.*—The di-tert-amylphenol-phosphorus pentoxide (3:1) product and mineral oil were mixed in a 2-liter, 4-necked, flask equipped with a condenser, thermometer and mechanically driven stirrer. Acetic acid was added followed by zinc oxide at room temperature and the reaction mixture heated to 155° C., during the course of which an aqueous acetic acid distillate was collected with the aid of a nitrogen flush. The reaction mixture was then held at 155° C. to 165° C. under diminished pressure for one hour. Upon cooling to 100° C. a slurry of water and magnesium hydroxide was added and the mixture heated to 165° C. during the course of two hours and held at this temperature for 1/4 hour under diminished pressure. The reaction product was then cooled to 100° C. and filtered through filtering clay contained on a heated Buchner funnel. The filtrate, representing the finished product, contained 1.48% magnesium, 7.41% zinc and 2.72% phosphorus.

## Example 8

DODECYLPHENOL-P<sub>2</sub>O<sub>5</sub> (3:1) PRODUCT

| Reaction mixture:             | Grams |
|-------------------------------|-------|
| Dodecylphenol                 | 600   |
| P <sub>2</sub> O <sub>5</sub> | 102.5 |

*Procedure.*—The dodecylphenol was placed in a 1-liter, 4-necked, round-bottom flask equipped with a reflux condenser, a thermometer and a mechanically driven stirrer and was heated with agitation to 100° C. and then phosphorus pentoxide was added portionwise, keeping the temperature constant, over a two-hour period. The temperature of the reaction mixture was then raised to 150° C. and maintained at 150° C. for three hours. The product contained 6.43% phosphorus and possessed an N. N. of 158.

## 9

## Example 9

COMPLEX ZINC ACETATE SALT OF DODECYLPHENOL-P<sub>2</sub>O<sub>5</sub> (3:1) PRODUCT

## Reaction mixture:

|                                                                                 |       |       |
|---------------------------------------------------------------------------------|-------|-------|
| Dodecylphenol-P <sub>2</sub> O <sub>5</sub> (3:1) product (N. N. = 158) (Ex. 8) | grams | 400   |
| Mineral oil (S. U. V. of 100 sec. at 100° F., acid-refined Mid-Continent)       | grams | 400   |
| Zinc oxide                                                                      | do    | 91.5  |
| Acetic acid (glacial)                                                           | do    | 136.0 |
| H <sub>2</sub> O                                                                | ml.   | 226.0 |

Procedure.—The dodecylphenol-phosphorus pentoxide (3:1) product and mineral oil were mixed in a 2-liter, 4-necked, round-bottom flask equipped with a thermometer, a Dean-Stark type distillation assembly, a submerged gas inlet tube, and a mechanically driven stirrer. Aqueous zinc acetate prepared by heating zinc oxide, acetic acid and water to 95° C. was added to the dodecylphenol-phosphorus pentoxide (3:1)-oil mixture at 85° C. The reaction mixture was heated to 165° C. with removal by distillation of dilute aqueous acetic acid with the aid of nitrogen bubbled through the gas inlet tube. On attaining 165° C., the reaction mixture was held at that temperature for 3/4 hour under atmospheric pressure and for 1/4 hour under diminished pressure to insure removal of acetic acid. The material was cooled to 100° C. and filtered through filtering clay contained on a heated Buchner funnel. The filtrate, representing the finished product, contained 7.27% zinc.

## Example 10

COMPLEXED MAGNESIUM-ZINC ACETATE SALT OF DODECYLPHENOL-P<sub>2</sub>O<sub>5</sub> (3:1) PRODUCT

## Reaction mixture:

|                                                                                        |       |      |
|----------------------------------------------------------------------------------------|-------|------|
| Acetate zinc salt of dodecylphenol-P <sub>2</sub> O <sub>5</sub> (3:1) product (Ex. 9) | grams | 439  |
| Mg(OH) <sub>2</sub>                                                                    | do    | 32.8 |
| H <sub>2</sub> O                                                                       | ml.   | 98.4 |

Procedure.—The acetate zinc salt of dodecylphenol-phosphorus pentoxide (3:1) product was placed in a 1-liter, 4-necked, round-bottom flask equipped with a thermometer, a Dean-Stark type distillation assembly, a submerged gas inlet tube and a mechanically driven stirrer and was heated with agitation to 85° C. An aqueous slurry was made from the Mg(OH)<sub>2</sub> and H<sub>2</sub>O, and was added at 25° C. to the zinc salt. Water was removed from the reaction by distillation with the aid of a stream of nitrogen, the reaction temperature attaining 165° C. after dehydration. The reaction was maintained at 165° C. for one hour at atmospheric pressure and then cooled to 100° C. and filtered through filtering clay contained on a heated Buchner funnel. The filtrate, representing the finished product, contained 1.7% magnesium, 6.29% zinc and 2.49% phosphorus.

## Example 11

C<sub>14</sub> ALKYLPHENOL-P<sub>2</sub>O<sub>5</sub> (3:1) PRODUCT

Reaction mixture: Grams

|                                          |      |
|------------------------------------------|------|
| C <sub>14</sub> alkylphenol <sup>2</sup> | 300  |
| P <sub>2</sub> O <sub>5</sub>            | 44.4 |

<sup>2</sup> "Oronite" alkylphenol No. 14, a mixture of monoalkylated phenols, consisting predominantly of para isomers, the alkyl groups of which are branch-chained and contain an average of about 14 carbon atoms.

Procedure.—The C<sub>14</sub> alkylphenol was placed in a 1-liter, 4-necked, round-bottom flask equipped with a reflux condenser, thermometer and mechanically driven stirrer and heated to 100° C. Phosphorus pentoxide was added during the course of one hour, the temperature then being raised to 150° C. and held there for four hours. The mixture was cooled and filtered through filtering clay contained on a heated Buchner funnel. The filtrate, representing the finished product, contained 5.43% phosphorus and had an N. N. of 148.

## 10

## Example 12

COMPLEX MAGNESIUM-ZINC ACETATE SALT OF C<sub>14</sub> ALKYLPHENOL-P<sub>2</sub>O<sub>5</sub> (3:1) PRODUCT

## Reaction mixture:

|                                                                                  |       |      |
|----------------------------------------------------------------------------------|-------|------|
| C <sub>14</sub> alkylphenol-P <sub>2</sub> O <sub>5</sub> (3:1) product (Ex. 11) | grams | 536  |
| Mineral oil (S. U. V. of 100 sec. at 100° F., acid-refined Mid-Continent)        | grams | 155  |
| Zinc oxide                                                                       | do    | 32.9 |
| Acetic acid (glacial)                                                            | do    | 48.7 |
| Magnesium hydroxide                                                              | do    | 23.6 |
| H <sub>2</sub> O                                                                 | ml.   | 176  |

Procedure.—The procedure was the same as that for Example 7. The product contained 1.33% magnesium, 5.63% zinc and 2.33% phosphorus.

## Example 13

WAX-PHENOL (3-14)-P<sub>2</sub>O<sub>5</sub> (3:1) PRODUCT

|                                                                          |       |
|--------------------------------------------------------------------------|-------|
| Reaction mixture:                                                        | Grams |
| Wax-phenol (3-14)                                                        | 1000  |
| Mineral oil (S. U. V. of 296 sec. at 100° F., solvent-refined Penna oil) | 2000  |
| P <sub>2</sub> O                                                         | 60    |

Procedure.—The wax-phenol (3-14) and mineral oil were placed in a 5-liter, 4-necked, round-bottom flask equipped with a reflux condenser, thermometer and mechanically driven stirrer and were warmed with agitation to 100° C. The phosphorus pentoxide was added portionwise at 100° C. over 2 1/2 hours, followed by a reaction period of 7 1/2 hours at 100° C. The clear amber colored reaction product was filtered through filtering clay contained on a heated Buchner funnel. The product was found to have an N. N. of 19.2 and a phosphorus content of 0.84%.

## Example 14

NORMAL ZINC SALT OF WAX-PHENOL (3-14)-P<sub>2</sub>O<sub>5</sub> (3:1)

|                                                                                                 |       |
|-------------------------------------------------------------------------------------------------|-------|
| Reaction mixture:                                                                               | Grams |
| Wax-phenol (3-14)-P <sub>2</sub> O <sub>5</sub> (3:1) product (similar to Ex. 13, N. N. = 17.6) | 1000  |
| ZnO                                                                                             | 12.7  |
| HC <sub>2</sub> H <sub>3</sub> O <sub>2</sub> (glacial)                                         | 18.6  |
| H <sub>2</sub> O                                                                                | 31.6  |

Procedure.—The wax-phenol (3-14)-phosphorus pentoxide (3:1) product was placed into a 3-liter, 4-necked, round-bottom flask equipped with a thermometer, a submerged gas inlet tube, a Dean-Stark type distillation assembly and a mechanically driven stirrer. Zinc oxide, acetic acid and water were heated to 95° C. to form an aqueous solution of zinc acetate which was added to the wax-phenol (3-14)-phosphorus pentoxide (3:1) product at 70° C. The reaction mixture was heated with agitation to 165° C. with recovery of aqueous acetic acid condensate and then reacted at 165° C. for 3/4 hour at atmospheric pressure followed by like treatment under diminished pressure for 1/4 hour to insure complete removal of acetic acid. This product was utilized in the unfiltered condition as the intermediate in Example 15.

## Example 15

COMPLEX BARIUM-ZINC SALT OF WAX-PHENOL (3-14)-P<sub>2</sub>O<sub>5</sub> (3:1) PRODUCT

|                                                                                     |       |
|-------------------------------------------------------------------------------------|-------|
| Reaction mixture:                                                                   | Grams |
| Zinc salt of wax-phenol (3-14)-P <sub>2</sub> O <sub>5</sub> (3:1) product (Ex. 14) | 500   |
| Ba(OH) <sub>2</sub> ·8H <sub>2</sub> O                                              | 49.5  |
| H <sub>2</sub> O                                                                    | 50.0  |

Procedure.—The zinc salt of wax-phenol (3-14)-phosphorus pentoxide (3:1) product was placed into a 1-liter, 4-necked, round-bottom flask equipped with a thermometer, a submerged gas inlet tube, a Dean-Stark type distillation assembly and a mechanically driven stirrer, and

## 11

was heated with agitation to 80° C. The aqueous solution of  $\text{Ba}(\text{OH})_2 \cdot 8\text{H}_2\text{O}$  at 80° C. was added and the reaction mixture heated with agitation in the presence of a stream of nitrogen, to 165° C. allowing distillation of the water. The temperature was held at 165° C. for 1½ hours to insure complete dehydration. After cooling to 100° C., 4% filtering clay was added and the product filtered through filtering clay contained on a heated Buchner funnel. The filtrate, representing the finished product, contained 3.1% barium and 0.81% zinc.

## Example 16

WAX-PHENOL (3-14)- $\text{P}_2\text{O}_5$  (3:1) PRODUCT

## Reaction mixture:

|                                                  |       |     |
|--------------------------------------------------|-------|-----|
| Wax-phenol (3-14) (phenol content=approx. 11.9%) | grams | 300 |
| $\text{P}_2\text{O}_5$                           | do    | 18  |
| Toluene                                          | ml.   | 300 |

Procedure.—The wax-phenol (3-14) and toluene were placed in a 2-liter, 4-necked, round-bottom flask containing a reflux condenser, thermometer and mechanically driven stirrer. After heating to 100° C., phosphorus pentoxide was gradually added to the mixture over a four-hour period. Following this, the temperature of the mixture was held at 100° C. for a period of eight hours to insure complete reaction. The product was then filtered through filtering clay and the filtrate was topped to 150° C. under diminished pressure to remove the toluene solvent. The residue, representing the finished product, contained 2.2% phosphorus and had a N. N. of 48.

## Example 17

NORMAL ZINC SALT OF WAX-PHENOL (3-14)- $\text{P}_2\text{O}_5$  (3:1) PRODUCT

## Reaction mixture:

|                                                                          |       |     |
|--------------------------------------------------------------------------|-------|-----|
| Wax-phenol (3-14)- $\text{P}_2\text{O}_5$ (3:1) product (Ex. 16)         | grams | 100 |
| $\text{Zn}(\text{C}_2\text{H}_3\text{O}_2)_2 \cdot 2\text{H}_2\text{O}$  | do    | 9.5 |
| Mineral oil (S. U. V. of 296 sec. at 100° F., solvent-refined Penna oil) | grams | 300 |
| Ethyl alcohol                                                            | ml.   | 100 |

Procedure.—The wax-phenol (3-14)-phosphorus pentoxide (3:1) product and the mineral oil were placed in a 2-liter, 4-necked, round-bottom flask equipped with a reflux condenser, thermometer and a mechanically driven stirrer. The zinc acetate di-hydrate was dissolved in the ethyl alcohol and the solution added to the other reactant at room temperature. The reaction mixture was heated, removing alcohol by distillation to 175° C., and held at that temperature for one hour. After cooling, the reaction product was dissolved in benzene and the solution filtered through a Büchner funnel packed with filtering clay. The zinc salt was recovered as the distillation residue by topping to 175° C. under diminished pressure. This material contained 0.78% zinc and 0.52% phosphorus.

## Example 18

COMPLEX ZINC ACETATE SALT OF WAX-PHENOL (3-14)- $\text{P}_2\text{O}_5$  (3:1) PRODUCT

## Reaction mixture:

|                                                                         |       |      |
|-------------------------------------------------------------------------|-------|------|
| Wax-phenol (3-14)- $\text{P}_2\text{O}_5$ (3:1) product (Ex. 13)        | grams | 400  |
| $\text{Zn}(\text{C}_2\text{H}_3\text{O}_2)_2 \cdot 2\text{H}_2\text{O}$ | do    | 30.6 |
| Ethyl alcohol, Formula 30                                               | ml.   | 175  |

Procedure.—The wax-phenol (3-14)-phosphorus pentoxide (3:1) product was added to a 1-liter, 4-necked, round-bottom flask equipped with a reflux condenser, thermometer and mechanically driven stirrer. The zinc acetate di-hydrate was dissolved in Formula 30 alcohol and the solution added to the reaction flask at 60° C. The reaction mixture was heated with agitation and a nitrogen flush to remove alcohol and aqueous acetic acid.

## 12

and then held at the attained temperature of 165° C. under diminished pressure for one hour. The reaction product was cooled to 90° C., filtering clay added, and the product filtered through filtering clay on a heated Buchner funnel. The filtrate, representing the finished product, was a dark amber liquid containing 2.64% zinc and 0.75% phosphorus.

## Example 19

10 COMPLEXED BARIUM-ZINC ACETATE SALT OF WAX-PHENOL (3-14)- $\text{P}_2\text{O}_5$  (3:1) PRODUCT

## Reaction mixture:

|                                                                                                                                                                                                     |       |     |
|-----------------------------------------------------------------------------------------------------------------------------------------------------------------------------------------------------|-------|-----|
| Complexed zinc acetate salt of wax-phenol (3-14)- $\text{P}_2\text{O}_5$ (3:1) product (similar to Ex. 18) (containing 63% mineral oil S. U. V. of 100 sec. at 100° F., acid-refined Mid-Continent) | grams | 857 |
| $\text{Ba}(\text{OH})_2 \cdot 8\text{H}_2\text{O}$                                                                                                                                                  | do    | 76  |
| $\text{H}_2\text{O}$                                                                                                                                                                                | ml.   | 75  |

Procedure.—The zinc acetate salt of wax-phenol (3-14)-phosphorus pentoxide (3:1) product was added to a 2-liter, 4-necked, round-bottom flask equipped with a condenser, thermometer and mechanically driven stirrer and heated to 80° C. The barium hydroxide octahydrate and water were added to the reaction flask. The water was removed by distillation with the aid of a nitrogen flush by heating to a temperature of 120° C. After cooling to 100° C., filtering clay was added and the product filtered through filtering clay contained on a heated Buchner funnel. The filtrate, representing the finished product, contained 3.32% barium and 1.87% zinc.

## Example 20

35 OCENOL- $\text{P}_2\text{O}_5$  (3:1) PRODUCT

|                        |       |
|------------------------|-------|
| Reaction mixture:      | Grams |
| Ocenol (octadecenol)   | 536   |
| $\text{P}_2\text{O}_5$ | 94.6  |

Procedure.—The ocenol was placed in a 1-liter, 4-necked, round-bottom flask equipped with a reflux condenser, a thermometer, and a mechanically driven stirrer, and was heated to 85° C. The phosphorus pentoxide was added portionwise at 15-minute intervals over a two-hour period. After completion of the phosphorus pentoxide addition, the reaction mixture was heated to and maintained at 100° C. with agitation for eight hours. The product, a viscous amber colored liquid, had a potentiometric N. N. of 196.

## Example 21

50 COMPLEX MAGNESIUM-ZINC SALT OF OCENOL- $\text{P}_2\text{O}_5$  (3:1) PRODUCT

|                                                                           |       |
|---------------------------------------------------------------------------|-------|
| Reaction mixture:                                                         | Grams |
| Ocenol- $\text{P}_2\text{O}_5$ (3:1) product (Ex. 20)                     | 100   |
| Mineral oil (S. U. V. of 100 sec. at 100° F., acid-refined Mid-Continent) | 100   |
| $\text{ZnO}$                                                              | 14.2  |
| Acetic acid (glacial)                                                     | 21.0  |
| $\text{H}_2\text{O}$                                                      | 35.0  |
| $\text{Mg}(\text{OH})_2$                                                  | 20.3  |
| $\text{H}_2\text{O}$                                                      | 61.0  |

Procedure.—The ocenol-phosphorus pentoxide (3:1) product and the dilution oil were placed in a 500-ml., 4-necked, round-bottom flask equipped with a distillation assembly, a submerged gas inlet tube, a thermometer and a mechanically driven stirrer. After heating the mixture to 70° C., aqueous zinc acetate, prepared from heating zinc oxide, acetic acid and water to 90° C., was added directly and heating was increased and nitrogen bubbled through the mixture removing aqueous acetic acid by distillation. The temperature rose to 165° C. in one hour and the reaction was continued for an additional one-half hour under diminished pressure to insure removal of acetic acid. On cooling to 80° C., an aqueous slurry of

$Mg(OH)_2$  was introduced into the unfiltered intermediate zinc salt with agitation. The reaction mixture was gradually heated to 165° C. and maintained there for one hour with nitrogen bubbling through it to facilitate distillation of water. The residual product was treated at 100° C. with 4% of filtering clay and filtered through 1% of filtering clay contained on a heated Buchner funnel. The filtered product contained 1.1% magnesium, 4.79% zinc and 3.04% phosphorus.

## EVALUATION OF PRODUCTS

In order to determine the suitability of the mixed-metal complex salts of the invention as detergents and antioxidants in lubricating oils, oil blends of the various complex salt products described herein were prepared and subjected to engine tests. The test used was the Lauson detergency test D-4. The results of these tests are summarized in Table I. As seen from the table, the mixed-metal complex salts greatly improve the detergent and antioxidant character of the oil.

## LAUSON DETERGENCY TEST D-4

This test determines the effectiveness of the lubricating oil in preventing fouling as measured by the cleanliness of rings, lands, ring grooves and piston skirts. Cleanliness ratings are based on a scale of from 100 to 0, a 100 rating signifying a perfectly clean condition and a 0 rating

representing the worst possible deposit condition. Bearing weight loss is also measured as supplemental data.

A single cylinder, 4-cycle, liquid cooled Lauson engine with splash lubrication and having a copper-lead bearing is used. The operating conditions are as follows:

|                                                    |          |      |
|----------------------------------------------------|----------|------|
| Oil temperature                                    | ° F.     | 220  |
| Jacket temperature                                 | ° F.     | 275  |
| Speed                                              | R. P. M. | 1825 |
| Brake load                                         | H. P.    | 1.6  |
| One-half throttle.                                 |          |      |
| 13-1 air-fuel ratio.                               |          |      |
| Oil added every 20 hours (one gallon sample used). |          |      |

15 The engine is inspected at the end of 20, 60 and 100 hours, the duration of the test being 100 hours. The fuel used is a controlled "Mobilgas Special" type blend gasoline (40% thermal +30% catalytically cracked +30% straight run +2.5 cc. TEL/gal.).

16 For ready comparison, the metal and phosphorus contents of the various mixed metal complex salts prepared and tested as described herein are shown in Table II. It will be seen that the phosphorus contents of the complex salts are about the same as the corresponding normal zinc salts, but that the metal content of the complex salts are much greater, generally at least about twice that of the normal salts.

TABLE I

| Example No. | Product                                                                                                         | Percent Additive | Percent Additive, Oil Free Basis | Lauson D-4 Piston Detergency Test (S. A. E. 20 Base Oil) <sup>1</sup> |          |           |          |                 |                          |            |  |
|-------------|-----------------------------------------------------------------------------------------------------------------|------------------|----------------------------------|-----------------------------------------------------------------------|----------|-----------|----------|-----------------|--------------------------|------------|--|
|             |                                                                                                                 |                  |                                  | Piston Cleanliness                                                    |          |           | Used Oil |                 | Bearing Wt. Loss (CU-PB) |            |  |
|             |                                                                                                                 |                  |                                  | 20 hours                                                              | 60 hours | 100 hours | N. N.    | K. V. @ 210° F. | Top, G.                  | Bottom, G. |  |
| 2           | Normal Zinc Salt of Octylphenol-P <sub>2</sub> O <sub>5</sub> (3:1) Product.                                    | None             |                                  | 69                                                                    | 68       | 58        | 2.8      | 12.14           | .290                     | .308       |  |
| 3           | Complex Calcium-Zinc Salt of Octylphenol-P <sub>2</sub> O <sub>5</sub> (3:1) Product.                           | 2.8              | 1.0                              | 78                                                                    | 69       | 63        | 2.3      | 10.48           | .067                     | .063       |  |
| 5           | Complexed Magnesium-Zinc Acetate Salt of Octylphenol-P <sub>2</sub> O <sub>5</sub> (3:1) Product.               | 1.8              | 1.0                              | 85                                                                    | 80       | 78        | 3.3      | 11.42           | .232                     | .163       |  |
| 7           | Complex Magnesium-Zinc Acetate Salt of di-tert-amylophenol-P <sub>2</sub> O <sub>5</sub> (3:1) Product.         | 1.6              | 1.0                              | 87                                                                    | 82       | 79        | 1.8      | 11.12           | .161                     | .125       |  |
| 10          | Complex Magnesium-Zinc Acetate Salt of Dodecylphenol-P <sub>2</sub> O <sub>5</sub> (3:1) Product.               | 1.0              | 0.5                              | 87                                                                    | 82       | 78        | 3.4      | 11.73           | .160                     | .148       |  |
| 12          | Complex Magnesium-Zinc Acetate Salt of C <sub>14</sub> Alkylphenol-P <sub>2</sub> O <sub>5</sub> (3:1) Product. | 0.85             | 0.5                              | 88                                                                    | 84       | 80        | 3.4      | 10.39           | .154                     | .141       |  |
| 17          | Normal Zinc Salt of Wax-Phenol (3-14)-P <sub>2</sub> O <sub>5</sub> (3:1) Product.                              | 4.0              | 1.0                              | 84                                                                    | 76       | 73        | 2.7      | 11.6            | .313                     | .299       |  |
| 15          | Barium-Zinc Salt of Wax-Phenol (3-14)-P <sub>2</sub> O <sub>5</sub> (3:1) Product.                              | 2.6              | 1.0                              | 92                                                                    | 86       | 81        | 4.3      | 12.27           |                          |            |  |
| 19          | Complexed Barium-Zinc Acetate Salt of Wax-Phenol (3-14)-P <sub>2</sub> O <sub>5</sub> (3:1) Product.            | 2.5              | 1.0                              | 87                                                                    | 80       | 73        | 2.5      | 12.15           | .126                     | .169       |  |
| 21          | Complex Magnesium Zinc Acetate Salt of Ocenol-P <sub>2</sub> O <sub>5</sub> (3:1) Product.                      | 1.8              | 1.0                              | 92                                                                    | 87       | 83        | 5.6      | 11.33           | .189                     | .189       |  |

<sup>1</sup> S. A. E. 20 Grade Solvent-Refined Penna Oil:

K. V. @ 100° F. 66.99  
K. V. @ 210° F. 8.69  
N. N. Nil

TABLE II

| Example No. | Product                                                                                                         | Theoretical Percent Metal For Normal Salt | Actual Percent Metal          | Percent Metal Equivalents in Excess of Theory | Percent Phosphorus |        |
|-------------|-----------------------------------------------------------------------------------------------------------------|-------------------------------------------|-------------------------------|-----------------------------------------------|--------------------|--------|
|             |                                                                                                                 |                                           |                               |                                               | Theory             | Actual |
| 3           | Complex Calcium-Zinc Salt of Octylphenol-P <sub>2</sub> O <sub>5</sub> (3:1) Product.                           | Zn-5.70                                   | Zn-4.26<br>Ca-2.60<br>Zn-9.85 | 48                                            |                    |        |
| 5           | Complex Magnesium-Zinc Acetate Salt of Octylphenol-P <sub>2</sub> O <sub>5</sub> (3:1) Product.                 | Zn-5.70                                   | Mg-2.34<br>Zn-7.41            | 182                                           | 3.45               | 3.38   |
| 7           | Complex Magnesium-Zinc Acetate Salt of di-tert-amylophenol-P <sub>2</sub> O <sub>5</sub> (3:1) Product.         | Zn-4.23                                   | Mg-1.48<br>Zn-6.29            | 257                                           | 2.62               | 2.72   |
| 10          | Complex Magnesium-Zinc Acetate Salt of Dodecylphenol-P <sub>2</sub> O <sub>5</sub> (3:1) Product.               | Zn-4.02                                   | Mg-1.74<br>Zn-5.63            | 172                                           | 2.82               | 2.49   |
| 12          | Complex Magnesium-Zinc Acetate Salt of C <sub>14</sub> Alkylphenol-P <sub>2</sub> O <sub>5</sub> (3:1) Product. | Zn-4.09                                   | Mg-1.33<br>Zn-0.81            | 209                                           | 2.35               | 2.33   |
| 15          | Barium-Zinc Salt of Wax-Phenol (3-14)-P <sub>2</sub> O <sub>5</sub> (3:1) Product.                              | Zn-0.96                                   | Ba-3.1<br>Zn-1.87             | 139                                           | 0.81               | 0.67   |
| 19          | Complexed Barium-Zinc Acetate Salt of Wax-Phenol-P <sub>2</sub> O <sub>5</sub> (3:1) Product.                   | Zn-0.95                                   | Ba-3.32<br>Zn-4.79            | 262                                           | 0.66               | 0.55   |
| 21          | Complex Magnesium Zinc Acetate Salt of Ocenol-P <sub>2</sub> O <sub>5</sub> (3:1) Product.                      | Zn-5.4                                    | Mg-1.1                        | 45                                            | 2.85               | 3.04   |

The amount of the mixed-metal complex salt to be incorporated into the lubricating oil generally will be within the range of from about 0.1 to about 10 weight percent, the usual amount being from about 0.25 to about 5 weight percent, i. e., on an oil-free basis.

As indicated hereinbefore, the products of the invention may be made up in the form of oil "concentrates." These concentrates will contain, as a rule, amounts of additives ranging from upwards of about 10 weight percent of the complex metal salt to the highest soluble concentration of the salt in the oil.

The compounds of this invention may be used in lubricating oil compositions containing other additives designed to improve the oil in different respects, e. g., E. P. agents, pour point depressants, V. I. improvers, defoamants, etc. The additives of the invention may also be used in oil in combination with other antioxidants and/or detergents.

While the preparation and utility of certain specific representative compounds have been described in detail herein, it is not intended that the invention be limited in any way thereby, but that it include such variations in procedures and such products as come within the spirit and scope of the accompanying claims.

What is claimed:

1. A mineral lubricating oil containing a minor proportion, sufficient to improve the detergent character thereof, of a mixed-metal, zinc-containing complex salt of a partial ester of phosphoric acid having a metal content greater than that which would be equivalent to the acid-hydrogen content of said partial ester prepared by the steps of (1) reacting one mol of phosphorus pentoxide with from about one to about three mols of an organic hydroxy compound selected from the group consisting of a hydroxy-aromatic compound that has an alkyl substituent having at least 8 carbon atoms in place of a nuclear hydrogen atom thereof and a primary, aliphatic alcohol having at least 8 carbon atoms per molecule, to form an acidic, partial ester of phosphoric acid, (2) reacting said acidic, partial ester of phosphoric acid with a zinc salt reagent in an amount sufficient to furnish at least one equivalent of zinc per equivalent of acid-hydrogen content in said acidic, partial ester of phosphoric acid, and (3) reacting the product obtained in step 2 with a metal hydroxide selected from the group consisting of calcium hydroxide, barium hydroxide, strontium hydroxide, cadmium hydroxide, magnesium hydroxide and cobalt hydroxide, in an amount sufficient to furnish at least one equivalent of metal per equivalent of acid-hydrogen content in said acidic, partial ester of phosphoric acid.

2. A mineral lubricating oil containing a minor proportion, sufficient to improve the detergent character thereof, of a mixed-metal, zinc- and calcium-containing complex salt of a partial ester of phosphoric acid having a metal content greater than that which would be equivalent to the acid-hydrogen content of said partial ester prepared by the steps of (1) reacting one mol of phosphorus pentoxide with from about one to about three mols of a hydroxy-aromatic compound having an alkyl substituent of at least 8 carbon atoms in place of a nuclear hydrogen atom thereof, to form an acidic, partial ester of phosphoric acid, (2) reacting said partial ester with an amount of zinc carbonate sufficient to provide about one equivalent of zinc per equivalent of acid-hydrogen content in said partial ester, and (3) reacting the product of step 2 with calcium hydroxide in an amount sufficient to provide about one equivalent of calcium per equivalent of acid-hydrogen in said partial ester.

3. A mineral lubricating oil containing a minor proportion, sufficient to improve the detergent character thereof, of a mixed-metal, zinc- and calcium-containing complex salt of a partial ester of phosphoric acid having a metal content greater than that which would be equivalent to the acid-hydrogen content of said partial ester, prepared by the steps of (1) reacting one mol of phos-

phorus pentoxide with about three mols of octylphenol, to form an acidic, partial ester of phosphoric acid, (2) reacting said partial ester with an amount of zinc carbonate to provide about one equivalent of zinc per equivalent of acid-hydrogen content in said partial ester, and (3) reacting the product of step 2 with calcium hydroxide in an amount sufficient to provide about one equivalent of calcium per equivalent of acid-hydrogen in said partial ester.

10 4. A mineral lubricating oil containing a minor proportion, sufficient to improve the detergent character thereof, of a mixed-metal, zinc-containing complex salt of a partial ester of phosphoric acid having a metal content greater than that which would be equivalent to the acid-hydrogen content of said partial ester, prepared by the steps of (1) reacting one mol of phosphorus pentoxide with from about one to about three mols of a hydroxy compound selected from a hydroxyaromatic compound having an alkyl substituent of at least 8 carbon atoms in

15 place of a nuclear hydrogen atom thereof and a primary, aliphatic alcohol, to form an acidic, partial ester of phosphoric acid, (2) reacting the partial ester formed in step 1 with an amount of zinc acetate sufficient to supply to the reaction at least about two equivalents of zinc per

20 equivalent of acid-hydrogen content in said partial ester, to form a complex zinc acetate salt of said partial ester, and (3) reacting the complex zinc acetate salt formed in step 2 with an amount of a metal hydroxide, the metal substituent of which is selected from the group consisting of calcium, barium, strontium, cadmium, magnesium and cobalt, sufficient to supply to the reaction an amount of metal at least equivalent to the acid-hydrogen content of said partial ester of phosphoric acid.

25 5. A mineral lubricating oil containing a minor proportion, sufficient to improve the detergent character thereof, of a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of

30 phosphorus pentoxide with from about one to about three mols of a hydroxyaromatic compound having an alkyl substituent of at least 8 carbon atoms in place of a nuclear hydrogen atom thereof, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

35 6. A mineral lubricating oil containing a minor proportion, sufficient to improve the detergent character thereof, of a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of C<sub>12</sub> alkylphenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex

40 zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

45 7. A mineral lubricating oil containing a minor proportion, sufficient to improve the detergent character thereof,

of a mixed-metal, zinc- and magnesium-containing complex salt of a partial ester of phosphoric acid having a metal content greater than that which would be equivalent to the acid-hydrogen content of said partial ester, prepared by the steps of (1) reacting one mole of phosphorus pentoxide with about three mols of C<sub>14</sub> alkylphenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2, in the presence of water, with an amount of magnesium hydroxide sufficient to supply to the reaction an amount of magnesium at least equivalent to the acid-hydrogen content of said partial ester of phosphoric acid.

8. A mineral lubricating oil containing a minor proportion, sufficient to improve the detergent character thereof, of a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of di-tertiary-*amyl*-phenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

9. A mineral lubricating oil containing a minor proportion, sufficient to improve the detergent character thereof, of a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with from about one to about three mols of an aliphatic alcohol having at least 8 carbon atoms, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

10. A mineral lubricating oil containing a minor proportion, sufficient to improve the detergent character thereof, of a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of *ocenol*, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

11. As a new composition of matter, a mixed-metal, zinc-containing complex salt of a partial ester of phosphoric acid having a metal content greater than that which would be equivalent to the acid-hydrogen content of said partial ester prepared by the steps of (1) reacting one mol of phosphorus pentoxide with from about one to about three mols of an organic hydroxy compound selected from the group consisting of a hydroxyaromatic compound that has an alkyl substituent having at least 8 carbon atoms in place of a nuclear hydrogen atom thereof and a primary, aliphatic alcohol having at least 8 carbon atoms per molecule, to form an acidic, partial ester of phosphoric acid, (2) reacting said acidic, partial ester of phosphoric acid with a zinc salt reagent in an amount sufficient to furnish at least one equivalent of zinc per equivalent of acid-hydrogen content in said acidic, partial ester, and phosphoric acid, and (3) reacting the product obtained in step 2 with a metal hydroxide selected from the group consisting of calcium hydroxide, barium hydroxide, strontium hydroxide, cadmium hydroxide, magnesium hydroxide and cobalt hydroxide, in an amount sufficient to furnish at least one equivalent of metal per equivalent of acid-hydrogen content in said acidic, partial ester of phosphoric acid.

12. As a new composition of matter, a mixed-metal, zinc- and calcium-containing complex salt of a partial ester of phosphoric acid having a metal content greater than that which would be equivalent to the acid-hydrogen content of said partial ester prepared by the steps of (1) reacting one mol of phosphorus pentoxide with from about one to about three mols of a hydroxy-aromatic compound having an alkyl substituent of at least 8 carbon atoms in place of a nuclear hydrogen atom thereof, to form an acidic, partial ester of phosphoric acid, (2) reacting said partial ester with an amount of zinc carbonate sufficient to provide about one equivalent of zinc per equivalent of acid-hydrogen content in said partial ester, and (3) reacting the product of step 2 with calcium hydroxide in an amount sufficient to provide about one equivalent of calcium per equivalent of acid-hydrogen in said partial ester.

13. As a new composition of matter, a mixed-metal, zinc- and calcium containing complex salt of a partial ester of phosphoric acid having a metal content greater than that which would be equivalent to the acid-hydrogen content of said partial ester, prepared by the steps of (1) reacting one mol of phosphorus pentoxide with about three mols of *octylphenol*, to form an acidic, partial ester of phosphoric acid, (2) reacting said partial ester with an amount of zinc carbonate to provide about one equivalent of zinc per equivalent of acid-hydrogen content in said partial ester, and (3) reacting the product of step 2 with calcium hydroxide in an amount sufficient to provide about one equivalent of calcium per equivalent of acid-hydrogen in said partial ester.

14. As a new composition of matter, a mixed-metal, zinc-containing complex salt of a partial ester of phosphoric acid having a metal content greater than that which would be equivalent to the acid-hydrogen content of said partial ester, prepared by the steps of (1) reacting one mol of phosphorus pentoxide with from about one to about three mols of a hydroxy compound selected from a hydroxyaromatic compound having an alkyl substituent of at least 8 carbon atoms in place of a nuclear hydrogen atom thereof and a primary, aliphatic alcohol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of a metal hydroxide, the metal substituent of which is selected from the group consisting of calcium, barium, strontium, cadmium, magnesium and cobalt, suf-

ficient to supply to the reaction an amount of metal at least equivalent to the acid-hydrogen content of said partial ester of phosphoric acid.

15. As a new composition of matter, a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with from about one to about three mols of a hydroxyaromatic compound having an alkyl substituent of at least 8 carbon atoms in place of a nuclear hydrogen atom thereof, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

16. As a new composition of matter, a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of C<sub>14</sub> alkylphenol, to form an acidic partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

17. As a new composition of matter, a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of C<sub>14</sub> alkylphenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2, in the presence of water, with an amount of magnesium hydroxide sufficient to supply to the reaction an amount of magnesium at least equivalent to the acid-hydrogen content of said partial ester of phosphoric acid.

18. As a new composition of matter, a mixed-metal,

zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of di-tertiary-amyphenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

19. As a new composition of matter, a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with from about one to about three mols of an aliphatic alcohol having at least 8 carbon atoms, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

20. As a new composition of matter, a mixed-metal, zinc- and magnesium-containing complex salt of a partial ester of phosphoric acid having a metal content greater than that which would be equivalent to the acid-hydrogen content of said partial ester, prepared by the steps of (1) reacting one mol of phosphorus pentoxide with about three mols of oenol, to form an acidic, partial ester of phosphoric acid, (2) reacting the partial ester formed in step 1 with an amount of zinc acetate sufficient to supply to the reaction at least about two equivalents of zinc per equivalent of acid-hydrogen content in said partial ester, to form a complex zinc acetate salt of said partial ester, and (3) reacting the complex zinc acetate salt formed in step 2 with an amount of magnesium hydroxide sufficient to supply to the reaction an amount of magnesium at least equivalent to the acid-hydrogen content of said partial ester of phosphoric acid.

#### References Cited in the file of this patent

#### UNITED STATES PATENTS

|           |            |               |
|-----------|------------|---------------|
| 2,228,659 | Farrington | Jan. 14, 1941 |
| 2,346,155 | Denison    | Apr. 11, 1944 |
| 2,378,800 | Amott      | June 19, 1945 |
| 2,745,863 | Otto       | May 15, 1956  |